# EUROPEAN PATENT SPECIFICATION

(11) **EP 2 868 758 B1**
(45) Date of publication and mention of the grant of the patent: **18.04.2018**
(21) Application number: 13813342.6
(22) Date of filing: 02.07.2013
(51) Int. Cl.: C22C 9/00, C22F 1/08, H01B 1/02, H01B 5/02, H01B 13/00

(54) **COPPER-ALLOY WIRE ROD AND MANUFACTURING METHOD THEREFOR**
KUPFERLEGIERUNGSWALZDRAHT UND HERSTELLUNGSVERFAHREN DAFÜR
FIL EN ALLIAGE DE CUIVRE, ET PROCÉDÉ DE FABRICATION DE CELUI-CI

(30) Priority: 02.07.2012 JP 2012148920
(43) Date of publication of application: 06.05.2015
(73) Proprietor: Furukawa Electric Co., Ltd., Chiyoda-ku Tokyo 100-8322 (JP)
(72) Inventor: TAKAZAWA, Tsukasa, Tokyo 100-8322 (JP)
(74) Representative: Forstmeyer, Dietmar
(86) International application number: PCT/JP2013/068160
(87) International publication number: WO 2014/007259

(56) References cited:
- WO-A1-2007/046378
- JP-A- 2001 234 309
- JP-A- 2003 237 428
- JP-A- 2008 095 202
- JP-A- 2009 280 860
- JP-A- 2009 280 860
- US-A1- 2002 066 503
- US-A1- 2004 238 086

## Description

### TECHNICAL FIELD

The present invention relates to a copper alloy wire and a method of producing the same, and more specifically the present invention relates to an extra-fine copper alloy wire for magnet wires and a method of producing the same.

### BACKGROUND ART

Along with the development in electronic equipment, making the size of an electronic part smaller is in progress, and there is an increasing demand for extra-fine copper alloy wire (round wire) having a wire diameter of 0.1 mm or less. For example, a coil for micro speakers that is used in mobile phones, smart phones, and the like, is produced by working an extra-fine wire (a magnet wire) having a wire diameter of 0.1 mm or less by winding into a coil shape.

For this winding, toughness (elongation) is required as the workability capable of turn formation, and pure copper excellent in toughness has been conventionally used. However, although pure copper is excellent in electrical conductivity, due to its low physical strength, there is a problem that pure copper is low in resistance to fatigue that is accompanied by coil vibration.

In order to solve this problem, there is a proposal of a technique of using a high-concentration Cu-Ag alloy containing 2 to 15 mass% of Ag that can enhance the tensile strength almost without lowering the electrical conductivity (Patent Literature 1). Furthermore, in general, a metal or an alloy, which has been subjected to working, is enhanced in tensile strength and lowered in elongation; however, when this is subjected to heating at a certain temperature or higher, elongation is recovered again, while physical strength is lowered. Thus, there is a proposal of a technique of achieving a balance between physical strength and elongation even in a low-concentration alloy, by carrying out the heating at a temperature lower than or equal to the softening temperature (Patent Literature 2). Furthermore, there is a proposal of a technology of enhancing resistance to bending fatigue, by applying compressive stress by subjecting a soft copper alloy wire with diameter φ2.6 mm and with electrical conductivity 98%IACS or more, to surface working (Patent Literature 3).

### CITATION LIST

### PATENT LITERATURES

Patent Literature 1: JP-A-2009-280860 ("JP-A" means unexamined published Japanese patent application)
Patent Literature 2: Japanese Patent No. 3941304
Patent Literature 3: JP-A-05-86445

US 2002/0066503 A1 discloses an ultrafine copper alloy wire with a diameter of not more than 0.08 mm, consisting of Cu, Ag and, optionally, Mg, In or Sn.

US 2004/0238086 A1 discloses a copper-magnesium alloy wire having high strength and high conductivity and a process for producing the same.

JP 2001 234309 A discloses an extra-fine copper alloy wire with an outer diameter of 0.01 to 0.08, which wire is produced from a copper alloy that consists of copper and a specified amount of a specified metal.

### SUMMARY OF INVENTION

### TECHNICAL PROBLEM

However, according to the demand for lengthening the service life of magnet wires and the demand for making magnet wires finer (with a wire diameter of 0.08 mm or less) as a result of making the size of electronic parts further smaller, further enhancement of resistance to bending fatigue and further strength enhancement of copper alloy wires has been demanded. As described in Patent Literature 1, when the Ag content is increased in order to further increase the physical strength, rather, electrical conductivity is lowered. Furthermore, since Ag is highly expensive, a noticeable increase in the cost is brought about. Furthermore, it is difficult to achieve further enhancement in physical strength and enhancement of resistance to bending fatigue, while securing electrical conductivity and elongation, using the conventional general solid solution-type highly electronic conductive copper alloy wire, as described in Patent Literature 2. Moreover, when it is intended to perform surface working so that the technology of Patent Literature 3 can be applied to a soft copper wire or copper alloy wire having a diameter of φ0.1 mm or less, since the soft copper wire or copper alloy wire having a diameter of φ0.1 mm or less has a markedly smaller wire diameter than the copper alloy wire described in Patent Literature 3, the strength of the copper alloy wire itself is low, and wire breakage occurs due to the load at the time of working, so that working itself is difficult to conduct.

Furthermore, recently, the shape of magnet wires is not limited to round wires, and investigations have also been conducted on the employment of square wires and rectangular wires. Even in the cases of these square wires and rectangular wires, it is requested to employ a wire with a thickness that is thin to the extent of that corresponding to the wire diameter of the round wire.

The present invention was achieved in view of the problems in those conventional art, and it is an object of the present invention to provide, at low cost, a copper alloy wire that is excellent in elongation, and resistance to bending fatigue, and that can be suitable for the use in, for example, magnet wires.

### SOLUTION TO PROBLEM

The inventors of the present invention conducted thorough investigations on various copper alloys, and heating and working conditions therefor, in order to develop a copper alloy wire that is superior in elongation, and resistance to bending fatigue, and that is suitably used in magnet wires, and the like. As a result, the inventors have found that when a copper alloy wire having a predetermined alloy composition is subjected to a semi-softening treatment, then the wire surface section is subjected to cold-working at a certain light working ratio, and thereby the hardness is increased to a predetermined level in a certain shallow range from the surface of the wire, a copper alloy wire having excellent elongation and resistance to bending fatigue can be obtained. The present invention was completed based on those findings.

That is, the present invention provides the following means:
(1) A copper alloy wire, having an alloy composition consisting of (i) 0.5 to 4 mass% of Ag and/or (ii) at least one selected from the group consisting of Sn, Mg, Zn, In, Ni, Co, Zr, and Cr each at a content of 0.05 to 0.3 mass%, with the balance being Cu and unavoidable impurities, wherein the copper alloy wire has a wire diameter (in the case of a round wire) or a wire thickness (in the case of a square wire or a rectangular wire) of 0.1 mm or less, and wherein the nanoindentation hardness in the wire surface section is 1.45 GPa or more as measured by nanoindenter ENT-2100 (manufactured by Elionix, Inc.), the wire surface section starting at the outermost surface of the wire and ranging at maximum to a distance from the surface that corresponds to 20% of the wire diameter or the wire thickness; the nanoindentation hardness at the center of the wire is less than 1.45 GPa as measured by nanoindenter ENT-2100 (manufactured by Elionix, Inc.), the tensile strength of the wire is 350 MPa or more, and the elongation is 7% or more.
(2) A method of producing the copper alloy wire of (1), containing the steps of:
   wire-working of subjecting a rough-drawn wire of a copper alloy having an alloy composition consisting of (i) 0.5 to 4 mass% of Ag and/or (ii) at least one selected from the group consisting of Sn, Mg, Zn, In, Ni, Co, Zr, and Cr each at a content of 0.05 to 0.3 mass%, with the balance being Cu and unavoidable impurities, to cold-working, to form a wire having a wire diameter or a wire thickness of 0.1 mm or less;
   final-heating, which is carried out in a batch mode at 300°C to 450°C for 30 minutes to 2 hours; or in a continuous mode at 300°C to 700°C for 0.5 to 5 seconds; and
   cold-working the wire that has been subjected to the heating, at a working ratio of 3 to 15%.
(3) The method of producing a copper alloy wire according to (2), wherein in the wire-working step, intermediate heating is carried out in the course of a plurality of cold-working steps so that the wire after this intermediate heating has a tensile strength of 330 MPa or more and an elongation of 10% or more.

Herein, in the present specification, a semi-softened state means a state in which elongation of the copper alloy wire satisfies 10% or more, preferably 10% to 30%. Also, a semi-softening treatment means a heating that brings about the semi-softened state. On the other hand, a softened state means a recovered state in which elongation of a copper alloy wire is more than 30%. Furthermore, a softening treatment means a heating at a high temperature that brings about the softened state.

In the present invention, a wire means to include a square wire or a rectangular wire, in addition to a round wire. Thus, unless otherwise specified, the wire of the present invention collectively means a round wire, a square wire, and a rectangular wire. Herein, the size of the wire means, in the case of a round wire (the cross-section in the transverse direction (TD) is circular), the wire diameter ϕ (the diameter of the circle of the cross-section) of the round wire; in the case of a square wire (the cross-section in the transverse direction is square), the thickness t and the width w (each being the length of one side of the square of the cross-section and being identical to each other) of the square wire; and in the case of a rectangular wire (the cross-section in the transverse direction is rectangular), the thickness t (the length of a shorter side of the rectangle of the cross-section) and the width w (the length of a longer side of the rectangle of the cross-section) of the rectangular wire.

### ADVANTAGEOUS EFFECTS OF INVENTION

Since the copper alloy wire of the present invention is excellent in resistance to bending fatigue, while having elongation necessary in coil-formation, the wire is preferably suitable as, for example, a copper alloy wire for magnet wires. Also, the method of producing the copper alloy wire of the present invention is preferably suitable as the producing method of the copper alloy wire, which is excellent in the performance.

### BRIEF DESCRIPTION OF DRAWING

{Fig. 1}
Fig. 1 is a front view schematically showing the apparatus used in the test for measuring the number of repeating times at breakage in bending fatigue (the number of repeating times at breakage), which was conducted in the Examples.

### MODE FOR CARRYING OUT THE INVENTION

The present invention will be described in detail below.

### [Hardness at surface portion of wire]

In regard to the copper alloy wire of the present invention, the nanoindentation hardness in the wire surface section is 1.45 GPa or more as measured by nanoindenter ENT-2100 (manufactured by Elionix, Inc.). According to the present invention, the wire surface section starts at the outermost surface of the wire and ranges at maximum to a distance from the outermost surface of the wire that corresponds to 20% of the wire diameter in the case of a round wire or the wire thickness in the case of a square wire or a rectangular wire. Preferably, the nanoindentation hardness in the wire surface section corresponding to 15% of the wire diameter or the wire thickness, is adjusted to 1.45 GPa or more. Herein, the region having the particular nanoindentation hardness is formed to acquire the hardness, by work hardening with a final (finish) working that is provided after the final heating resulting in a semi-softened state. In the present specification, the wire surface section is also referred to as "surface worked layer" or "depth region extending from the outermost surface of the wire toward the inner side of the wire diameter or the wire thickness". Also, the center of the wire has a nanoindentation hardness of less than 1.45 GPa as measured by nanoindenter ENT-2100 (manufactured by Elionix, Inc.), and the wire as a whole is not
hardened like the wire surface section. According to the present invention, the reason why the region having a nanoindentation hardness of 1.45 GPa or more is set to extend from the outermost surface of the wire toward 20% inner side at the maximum of the wire diameter or the wire thickness, is that if the wire is hardened to a deeper region beyond this range (toward the center side of the wire), elongation cannot be sufficiently secured.

Furthermore, on the side closer to the center than this surface worked layer, the wire is in the semi-softened state as a result of the final heating and is not hardened. The nanoindentation hardness on the inner side than the surface worked layer (representatively, the central section of the wire) is usually less than 1.45 GPa, and in order to sufficiently secure elongation, the nanoindentation hardness is preferably 1.3 GPa or less.

Herein, the nanoindentation hardness means the hardness that can be determined by a method for measuring the hardness of a microscopic region, which is called a nanoindentation method, by pressing a triangular pyramid diamond indenter against the surface of a (wire) sample, and determining the hardness from the load exerted at that time and the contact projection area between the indenter and the sample. Between the nanoindentation hardness and the Vickers hardness, which is a general index of hardness, for example, the relationship of Vickers hardness = (76.2 × nanoindentation hardness) + 6.3 is known (Non-Patent Literature 1).

Non-Patent Literature 1: Kinzoku (Metal), Vol. 78 (2008) No. 9, p. 47

In regard to the copper alloy wire of the present invention, the wire surface section is formed as a work-hardened surface worked layer, and the resistance to bending fatigue of the wire can be further enhanced by adjusting the nanoindentation hardness at this wire surface section preferably to 1.5 GPa or more. Furthermore, when the thickness of the surface worked layer in which this predetermined nanoindentation hardness is 1.5 GPa or more is a depth region extending from the outermost surface of the wire toward at least 5% inner side of the wire diameter or the wire thickness (a depth region extending toward 20% inner side at the maximum, and preferably a depth region extending toward 15% inner side), satisfactory characteristics, such as an elongation of 10% or more, for the copper alloy wire as a whole can be exhibited. Therefore, an excellent magnet wire can be obtained.

In regard to the copper alloy wire of the present invention, the nanoindentation hardness at the wire surface section is set to 1.45 GPa or more; however, it is more preferable to set the nanoindentation hardness to 1.6 GPa or more. The upper limit is not particularly limited, but is usually set to 1.7 GPa or less.

### [Alloy composition]

The copper alloy wire of the present invention contains (i) Ag at a content of 0.5 to 4 mass%, and/or (ii) at least one selected from the group consisting of Sn, Mg, Zn, In, Ni, Co, Zr, and Cr each at a content of 0.05 to 0.3 mass%, with the balance being Cu and unavoidable impurities. Herein, when the content of an alloy additive element is simply expressed in "percent (%)", this means "mass%". Also, there are no particular limitations on the total content of at least one alloy component selected from the group consisting of Sn, Mg, Zn, In, Ni, Co, Zr, and Cr; however, in order to prevent a noticeable decrease in the electrical conductivity of the copper alloy wire, the total content of at least one alloy component selected from the group consisting of Sn, Mg, Zn, In, Ni, Co, Zr, and Cr, in addition to Ag, is preferably 0.5 mass% or less.

The copper alloy wire of the present invention may contain (i) Ag alone, or may contain (ii) at least one selected from the group consisting of Sn, Mg, Zn, In, Ni, Co, Zr, and Cr alone, or may contain both (i) Ag and (ii) at least one selected from the group consisting of Sn, Mg, Zn, In, Ni, Co, Zr, and Cr.

These elements each are a solid solution strengthening-type or precipitation strengthening-type element, and when any of these elements is/are added to Cu, physical strength can be enhanced without lowering the electrical conductivity to a large extent. As a result of this addition, the physical strength of the copper alloy wire itself is enhanced, and the resistance to bending fatigue is enhanced. Also, even if the wire is worked into an extra-fine wire having a wire diameter or a wire thickness of 0.1 mm or less, followed by subjecting to a heating (semi-softening treatment), since the wire surface section is hardened after the semi-softening treatment, the wire can withstand the final (finish) cold-working. Although the resistance to bending fatigue is generally proportional to tensile strength, if further working is applied in order to enhance the tensile strength, elongation is lowered, and the wire cannot be formed into an extra-fine copper alloy wire, such as a magnet wire. Herein, the bending strain exerted on the copper alloy wire at the time of bending fatigue increases toward the outer circumference of the wire, and the amount of bending strain decreases as the center is approached. Thus, according to the present invention, the resistance to bending fatigue can be enhanced, by work hardening the copper alloy wire by finish cold-working such that only a predetermined depth region (the wire surface section) of the wire surface has a predetermined hardness. Furthermore, while only the wire surface section is work-hardened, the entirety of the remaining portion of the wire other than the wire surface section (that is, the portion toward the deeper core than the predetermined depth, other than the wire surface section) maintains a semi-softened state. Thus, since elongation of the wire as a whole can be sufficiently secured, forming into an extra-fine copper alloy wire, such as a magnet wire, is enabled.

Among these elements, Ag is an element that can particularly enhance physical strength without lowering electrical conductivity, and is an exemplary essential additive element for the copper alloy related to the present invention used in, for example, magnet wires. In the present invention, the Ag content is set to 0.5 to 4.0 mass%, and preferably 0.5 to 2.0 mass%. If the content of Ag is too small, sufficient physical strength cannot be obtained. Also, if the Ag content is too large, electrical conductivity is lowered, and also it becomes excessively high cost.

The at least one element selected from the group consisting of Sn, Mg, Zn, In, Ni, Co, Zr, and Cr is an another example of an essential alloying element in the copper alloy according to the present invention. In the present invention, the contents of those elements are, respectively, 0.05 to 0.3%, and preferably 0.05 % to 0.2%. If this content is too small as the respective content, the effect of strength enhancement owing to the addition of any of these elements cannot be expected in most cases. Also, if this content is too large, since the lowering of the electrical conductivity is too large, the resultant copper alloy is inappropriate as a copper alloy wire, such as a magnet wire.

### [Production method]

The production method of the copper wire of the present invention will be described.

As discussed above, the shape of the copper alloy wire of the present invention is not limited to a round wire, and may also be a square wire or a rectangular wire. Then, these will be described below.

### [Production method of a round wire]

First, the method of producing a copper alloy round wire of the present invention is carried out by performing the steps, for example, of: casting; intermediate cold-working; intermediate heating (intermediate annealing); final-heating (final-annealing); and finish cold-rolling, in this order. Herein, when a copper alloy wire having desired properties can be obtained without being subjected to any intermediate annealing, the intermediate annealing may be omitted.

### [Casting]

To Cu, Ag and/or at least one additive element selected from the group consisting of Sn, Mg, Zn, In, Ni, Co, Zr, and Cr is/are added, and cast in a casting machine having the interior (internal walls) preferably made of carbon, for example, in a graphite crucible. The atmosphere inside the casting machine at the time of melting is preferably selected to be a vacuum or an inert gas atmosphere, such as nitrogen or argon, in order to prevent occurrence of oxides. There are no particular limitations on the casting method, and use may be made, for example, of a transverse continuous casting machine or an upcast method. By means of such a continuous casting wire-drawing method, steps can be carried out continuously from casting to wire-drawing, and a roughly-drawn rod is cast with a diameter of generally about φ 8 to 23 mm.

In the case where no continuous casting wire-drawing method is utilized, a roughly-drawn rod having a diameter of generally about φ 8 to 23 mm is similarly obtained, by subjecting the billet (casting ingot) obtained by casting, to wire-drawing.

### [Cold-working, intermediate annealing] (wire-working steps)

When this roughly-drawn rod is subjected to cold-working, the roughly-drawn rod is worked into a fine diameter wire having a diameter of φ 0.1 mm or less. Regarding this cold-working, it is preferable to perform cold wire-drawing.

The working ratio in this cold-working (wire-drawing) may vary depending on the target wire diameter, the copper alloy composition, and the heating or cold-working conditions thereafter, and there are no particular limitations. The working ratio is generally set to 70.0 to 99.9%.

When this cold-working includes a plurality of cold-working steps, such as first cold-working (wire-drawing) and second cold-working (wire-drawing), intermediate annealing (intermediate heating) may be carried out in the mid course of the first cold-working and the second cold-working.

The heating method of performing the intermediate annealing may be roughly classified into a batch-type method and a continuous method. Since the batch-type heating requires a longer treatment time period and a larger cost, this method is rather poor in productivity. However, since it is easy to perform the control of temperature or retention time period, it is easy to perform the control of characteristics. On the contrary, since the continuous-type heating can carry out heating and the wire-drawing continuously, this is excellent in productivity. However, since it is necessary to perform this heating in a very short time period, it is necessary to precisely control the heating temperature and time period, to realize characteristics stably. Those heating methods have advantages and disadvantages as described above, and therefore, it is desirable to select the heating method according to the purpose.

In the case of the batch-type heating, for example, it is preferable to perform heating in a heating furnace in an inert atmosphere, such as nitrogen or argon, at 300°C to 600°C for 30 minutes to 2 hours.

Examples of the continuous-type heating include an electrically heating-type heating and an in-atmosphere running-type heating. The electrically heating-type heating is a method of: providing electrode rings in the mid course of the wire-drawing step; passing an electric current to the copper alloy wire that passes among the electrode rings; and performing heating by the Joule heat generated by the copper alloy wire itself. The in-atmosphere running-type heating is a method of: providing a vessel for heating in the mid course of wire-drawing; and performing heating by passing a copper alloy wire in the atmosphere of the vessel for heating that has been heated to a predetermined temperature (for example, 300°C to 700°C). For both of those heating methods, it is preferable to perform heating in an inert gas atmosphere, in order to prevent oxidation of the copper alloy wire. In the case of the continuous-type, it is preferable to perform the heating at 300° to 700°c for 0.5 to 5 seconds.

By performing the intermediate annealing in the mod course of a plurality of cold-working steps, elongation of the wire thus obtainable can be recovered, and thereby workability can be enhanced. Also, Ag precipitation is accelerated by the intermediate annealing, and thus the physical strength and electrical conductivity of the wire thus obtainable can be further enhanced. For example, it is preferable to carry out the intermediate annealing under the conditions that satisfy the characteristics of a tensile strength of 330 MPa or more and an elongation of 10% or more of the copper alloy wire after this intermediate heating.

### [Finish-annealing (also referred to as final-annealing)] (final-heating step)

The copper alloy wire that has been worked to a desired size (wire diameter) by the steps described above, is subjected to finish-annealing as the final-heating.

The heating as the finish-annealing is carried out under the conditions that satisfy the characteristics of a tensile strength of 330 MPa or more and an elongation of 10% or more of the copper alloy wire after the heating. When the finish-annealing is carried out by such a semi-softening treatment, the physical strength of the copper alloy wire itself is enhanced, the resistance to bending fatigue is enhanced, and it can be made easier to perform finish cold-working on the surface after the heating.

Examples of the heating method of conducting finish-annealing include, similarly to the intermediate annealing, a batch-type heating and a continuous-type heating.

At the time of this finish-annealing, the tensile strength and elongation in the wire after the final-heating may undergo slight changes, depending on the composition of copper alloy wire or the working ratio. Thus, in the present invention, the heating temperature and the heating retention time period for the final heating (the finish-annealing) are appropriately adjusted such that the tensile strength of 330 MPa or more and the elongation would be 10% or more of the copper alloy wire obtainable by this finish-annealing.

In general, as the heating temperature is higher, the heating is carried out for a shorter time period, and as the heating temperature is lower, the heating is carried out for a longer time period. According to the present invention, when the finish-annealing is carried out in a batch mode, the heating is carried out at 300°C to 450°C for 30 minutes to 2 hours. On the other hand, when the finish-annealing is carried out in a continuous mode, the heating is carried out at 300°C to 700°C for 0.5 to 5 seconds.

The finish-working is carried out after this final-annealing. The characteristics of the copper alloy wire before the final-annealing are adjusted, and the final-annealing conditions are determined, as described above, so that the final characteristics of the copper alloy wire obtainable by the finish cold-working after this final-annealing give a tensile strength of 350 MPa or more and an elongation of 7% or more.

### [Finish cold-working] (cold-working step)

The copper alloy wire that has been subjected to the final-heating described above is subjected to final (finish) cold-working, and thereby the copper alloy wire is hardened so as to obtain a nanoindentation hardness at the wire surface section of 1.45 GPa or more. Since the copper alloy wire of the present invention has high strength, even an extra-fine wire having a wire diameter φ or a wire thickness t of 0.1 mm or less can be subjected to finish cold-working. In general, the resistance to bending fatigue is proportional to tensile strength; however, when working is further applied in order to enhance the tensile strength, elongation is lowered, and the wire cannot be formed into a magnet wire or the like. The bending strain exerted on the wire at the time of bending fatigue increases toward the outer circumference of the wire, and the amount of bending strain decreases as the center is approached. Thus, the resistance to bending fatigue can be enhanced, by hardening only the wire surface section by performing finish cold-working. Furthermore, since only the wire surface section of the wire is hardened while the center side of the wire maintains a semi-softened state, elongation of the wire as a whole can be sufficiently secured, and forming into an extra-fine wire, such as a magnet wire, is also enabled. According to the present invention, the risk of wire breakage can be effectively decreased, by performing a semi-softening heating that gives characteristics of a strength of 350 MPa or more and an elongation of 7% or more in the copper alloy wire of the final product, before the wire is subjected to finish cold-working. As this finish cold-working, wire-drawing work is carried out, and the working ratio of this wire-drawing is usually 3 to 15%, preferably 5 to 15%, and more preferably 7 to 12%. If the working ratio of this finish cold-working is too low, the surface working and strength are insufficient, and the effect of enhancing the resistance to bending fatigue may be insufficient. Furthermore, if the working ratio of this finish cold-working is too high, the relevant working affects the entirety of the wire beyond the wire surface section, so that elongation is impaired, and also the risk of wire breakage in working may be increased.

### [Production method of a rectangular wire]

Next, the method of producing a copper alloy rectangular wire of the present invention is the same as the method of producing a round wire described above, except for containing rectangular wire-working, and that finish cold-working appropriate for a rectangular shape is carried out. Specifically, the method of producing a rectangular wire of the present invention is carried out by performing steps of, for example, casting; intermediate cold-working (cold-wire-drawing); rectangular wire-working; final-heating (final-annealing); and finish cold-working, in this order. It is also the same as the method of producing a round wire from the viewpoint that if necessary, intermediate annealing (intermediate heating) is included between the intermediate cold-working and the rectangular wire-working. The conditions of the working/heating for the steps, such as casting, cold-working, intermediate annealing, and final-annealing, and preferred conditions thereof are also the same as those for the method of producing a round wire.

### [Rectangular wire-working]

Up to the steps before the rectangular wire-working, the production work is the same as that for the round wire, in which an ingot obtained by casting is subjected to cold-working (wire-drawing) to obtain a roughly-drawn rod having a round wire shape, and the roughly-drawn rod is further subjected to intermediate annealing if necessary. Regarding the rectangular wire-working, the round wire (roughly-drawn rod) thus obtained is subjected to cold rolling using a rolling machine, cold rolling using a cassette roller die, pressing, drawing, and the like. Through this rectangular wire-working, the transverse direction (TD) cross-section shape is worked into a rectangular shape, to obtain the shape of a rectangular wire. This rolling and the like are generally carried out in one to five passes. The reduction ratio in each pass and the total reduction ratio at the time of rolling and the like are not particularly limited, and may be appropriately set to obtain a desired rectangular wire size. Herein, the reduction ratio is the ratio of change in the thickness in the rolling direction upon performing the rectangular wire-working, and when the thickness before rolling is designated as t₁, and the thickness of the wire after rolling is designated as t₂, the reduction ratio (%) is represented by: {1 - (t₂/t₁)) × 100. For example, this total reduction ratio can be adjusted to 10 to 90%, and the reduction ratio in each pass can be adjusted to 10 to 50%. Herein, in the present invention, there are no particular limitations on the cross-section shape of the rectangular wire, but the aspect ratio is generally 1 to 50, preferably 1 to 20, and more preferably 2 to 10. The aspect ratio (represented by w/t as described below) is the ratio of a shorter side to a longer side in the rectangle that forms the transverse direction (TD) cross-section of a rectangular wire. In regard to the size of the rectangular wire, a rectangular wire thickness t is equal to the shorter side of the rectangle that forms the transverse direction (TD) cross-section, and a rectangular wire width w is equal to the longer side of the rectangle that forms the transverse direction (TD) cross-section. The rectangular wire thickness is generally 0.1 mm or less, preferably 0.08 mm or less, and more preferably 0.06 mm or less. The rectangular wire width is generally 1 mm or less, preferably 0.7 mm or less, and more preferably 0.5 mm or less.

### [Finish cold-working]

Finish cold-working is carried out, in the case of a rectangular wire, in the same manner as in the rectangular wire-working. It is the same as in the case of a round wire that the rectangular wire is hardened by this finish cold-working so as to obtain a nanoindentation hardness of the wire surface section of 1.45 GPa or more. Specifically, the finish cold-working on the rectangular wire is carried out by cold rolling using a rolling machine, or cold rolling using a cassette roller die. This working ratio is usually 3 to 15%, preferably 5 to 15%, and more preferably 7 to 12%. If the working ratio of this finish cold-working is too low, surface working and strength are insufficient, and the effect of enhancing the resistance to bending fatigue may be insufficient. Furthermore, if the working ratio of this finish cold-working is too high, the relevant working affects the entirety of the wire beyond the wire surface section, elongation is impaired, and the risk of wire breakage in working may be increased.

A rectangular wire produced by such working and heating is provided with a hardened layer having a nanoindentation hardness of 1.45 GPa or more as a surface worked layer by finish cold-working, in a region extending from the wire surface toward at least 5% in depth (a region extending from the wire surface toward 20% in depth at the maximum, and preferably a region extending from the wire surface toward 15% in depth) in the upper and lower surface layers in the thickness direction. A difference lies in that in the case of the round wire, the hardened layer is retained at the surface worked layer over the entire surface of the wire in the circumferential direction, while in the case of the rectangular wire, the hardened layer is retained as the surface worked layer respectively on the upper surface and the lower surface in the thickness direction at the surface of the wire. However, the round wire and the rectangular wire (and the square wire) have a common factor that the hardened layer is retained as the surface worked layer in the wire surface section in a predetermined shallow range.

When this rectangular wire is subjected to coil working in the thickness direction, high elongation and high bending fatigue characteristics can be exhibited, similarly to the round wire according to the present invention. Herein, subjecting a rectangular wire to coil working in the thickness direction implies winding a rectangular wire into a coil shape while taking the width w of the rectangular wire as the width of the coil.

### [Production method of a square wire]

Furthermore, in the case of producing a square wire, it is enough to set the transverse direction (TD) cross-section to be a square (w = t), in the method of producing a rectangular wire.

### [Another embodiment of the production method of a wire]

Another embodiment of the method of producing a copper alloy wire of the present invention may be a whole production process of: first subjecting a roughly-drawn rod obtained by casting to first cold-working (wire-drawing); recovering elongation by intermediate annealing; further performing second cold-working (wire-drawing) to obtain a desired wire diameter or a desired wire thickness; and controlling a predetermined mechanical strength and elongation by final (finish) annealing; and then adjusting the nanoindentation hardness of the wire surface section by final (finish) cold-working, while simultaneously finally adjusting the entire copper alloy wire so as to have predetermined mechanical strength and elongation. However, it is preferable to reduce the number of cold-working steps, from the viewpoints of energy consumption and efficiency.

The respective working ratios for these first and second cold wire-drawings vary depending on the target wire diameter or wire thickness, the copper alloy composition, and the conditions for the two heating of intermediate annealing and finish-annealing, and there are no particular limitations on the working ratios. However, generally, the working ratio for the first cold-working (wire-drawing) is set to 70.0 to 99.9%, and the working ratio for the second cold-working (wire-drawing) is set to 70.0 to 99.9%.

### [Other embodiments of the production methods of a rectangular wire and a square wire]

Instead of the production method described above, a sheet or a strip having a predetermined alloy composition is produced, and the sheet or strip is slit, to obtain a rectangular wire or square wire having a desired wire width.

This production process, for example, contains: casting, hot-rolling, cold-rolling, finish-annealing, finish cold-working, and slitting. If necessary, the intermediate annealing may be carried out in the middle of a plurality of cold rollings. Slitting may be carried out before the finish-annealing, or before the finish cold-working.

According to the production method described above, a copper alloy wire having a tensile strength of 350 MPa or more and an elongation of 7% or more is obtained.

### [Wire diameter or wire thickness, usage]

There are no particular limitations on the wire diameter or the wire thickness of the copper alloy wire of the present invention. The wire diameter or the wire thickness is preferably 0.1 mm or less, more preferably 0.08 mm or less, and even more preferably 0.06 mm or less. There are no particular limitations on the lower limit of the wire diameter or the wire thickness. At the current level of technique, the lower limit is generally 0.01 mm or more.

The use of the copper alloy wire of the present invention is not particularly limited. Examples of the use include an extra-fine magnet wire, for example, of a magnet wire, for use in speaker coils that are used in mobile telephones, smart phones, and the like.

### [Other physical properties]

The tensile strength of the copper alloy wire of the present invention is set to 350 MPa or more, because, if the tensile strength is less than 350 MPa, the strength is insufficient when the diameter is made finer by wire-drawing, and the wire is poor in resistance to bending fatigue.

Furthermore, the elongation of the copper alloy wire of the present invention is set to 7% or more, because, if the elongation is less than 7%, the wire is poor in workability, and the resultant wire is occurred with defects, such as wire breakage, at the time of forming into a coil.

The copper alloy wire of the present invention obtained by the above method exhibits high resistance to bending fatigue and exhibits elongation that enables forming into an extra-fine copper alloy wire, such as an extra-fine magnet wire.

### EXAMPLES

The present invention will be described in more detail based on examples given below, but the invention is not meant to be limited by these.

### [Examples and Comparative examples of round wires]

With respect to the cast material, the copper alloys in Examples according to this invention having the respective alloy composition, as shown in Tables 1 to 3, each containing Ag at a content of 0.5 to 4 mass%, and/or at least one selected from the group consisting of Sn, Mg, Zn, In, Ni, Co, Zr, and Cr each at a content of 0.05 to 0.3 mass%, with the balance being Cu and unavoidable impurities; and the copper alloys in Comparative examples having the respective alloy composition as shown in Tables 1 to 3, were cast into roughly-drawn rods with diameters φ 10 mm, respectively, by a transverse-type continuous casting method.

Those roughly-drawn rods were subjected to cold-working (wire-drawing), intermediate annealing, finish-annealing, and finish cold-working (wire-drawing) (the total working ratio of the following first and second cold-working steps: 99.984%), to give round wire samples to have the final wire diameter of φ 40 µm for the Test Examples of Table 1 and Table 3, and to have the wire diameters indicated for the Test Examples of Table 2.

The heating of intermediate annealing and finish-annealing were carried out by any manner selected from three patterns of batch annealing, electric current annealing, and running annealing, each under a nitrogen atmosphere. The intermediate annealing was carried out only once in the mid course of the first cold-working (wire-drawing) and the second cold-working (wire-drawing). In the Test Examples indicated in Table 1 and Table 2, the intermediate annealing was not conducted in Test Examples. Furthermore, in the Test Examples indicated in Table 3, the intermediate annealing was conducted in some Test Examples, while not conducted in the other Test Examples. The wire diameter before the intermediate annealing after the first cold-working (wire-drawing) in the Test Examples in which intermediate annealing was carried out, is presented in the column "Wire diameter (mm)" of "Intermediate annealing" in Table 3. Regarding the working ratio of this case, the working ratio of the first cold-working (wire-drawing) was adjusted to 70.0 to 99.9%, and the working ratio of the second cold-working (wire-drawing) was adjusted to 70.0 to 99.9%.

The production conditions for the copper alloy round wires according to the present invention and the copper alloy round wire of Comparative examples, and the characteristics of the copper alloy round wires thus obtained, are presented in Tables 1 to 3.

### [Examples and Comparative examples of rectangular wires]

Rectangular wire samples were produced in the same manner as the above round wires, except that rectangular wire-working was carried out after the roughly-drawn rods were subjected to cold-working (wire-drawing), or after intermediate annealing if performed, then finish-annealing was carried out, and then finish cold-working was carried out. As shown in Table 4, some samples were subjected to intermediate annealing, and the other samples were not subjected to intermediate annealing.

Regarding the rectangular wire-working, as shown in Table 4, a round wire before this working was worked by cold rolling into a rectangular wire such that the wire diameter φ (mm) was worked into a size of width w (mm) × thickness t (mm). The finish cold-working was carried out by cold rolling, in the same manner as in the rectangular wire-working, except that the working ratios, as indicated in Table 4.

The production conditions for the copper alloy rectangular wires according to the present invention and the copper alloy rectangular wires of Comparative examples, and the characteristics of the copper alloy rectangular wires thus obtained, are presented in Table 4.

### [Characteristics/Physical properties]

With respect to the thus-obtained samples of the round wires and rectangular wires, various characteristics were tested and evaluated.

The tensile strength (TS) and elongation (EI) were measured, according to JIS Z2201 and Z2241.

The number of repeating times at breakage in bending fatigue was obtained by measuring the number of repeating times until the test specimen of wire broke in a bending fatigue test, using the apparatus illustrated in Fig. 1. As illustrated in Fig. 1, a test specimen of a copper alloy wire sample with a wire diameter φ or wire thickness t of 0.04 mm (40 µm) was sandwiched between two dies, and a load was applied thereon by hanging a weight (W) of 10 g at the lower end of the specimen in order to suppress deflection (flexure) of the wire. In the case of the rectangular wire, the sample was mounted to be sandwiched between the two dies in the wire thickness direction (ND). The upper end of the specimen was fixed with a connecting jig. While having the specimen maintained in this state, the specimen was bended 90° on the left side and the right side, respectively, bending was repeatedly carried out at a speed of 100 times per minute, and the number of repeating times at breakage in bending was measured for each specimen, i.e. the respective sample. Regarding the number of repeating times in bending, one reciprocation of 1 → 2 → 3 in Fig. 1 was counted as one time, and the distance between the two dies was set to 1 mm so that the specimen of the copper alloy wire would not be compressed in the test. Determination of breakage was made such that the specimen was judged to be broken when the weight hung at the lower end of the specimen dropped. Furthermore, the radius of bending (R) was set to 2 mm, depending on the curvature of the dies.

The service life of a coil was evaluated as follows, based on the number of repeating times at breakage in bending fatigue measured by the test method described above. From the results of the bending fatigue test, a sample which had the number of times at breakage of 7,000 or more times was rated as "○○(excellent)", a sample which had the number of times at breakage of 5,000 times or more but less than 7,000 times was rated as "○ (good)", a sample which had the number of times at breakage of 3,000 times or more but less than 5,000 times was rated as "Δ (slightly poor)", and a sample which had the number of times at breakage of less than 3,000 times was rated as "× (poor)".

The wire-drawing property was evaluated by the presence or absence of wire breakage in wire-drawing. In this test, a test of subjecting a copper alloy wire that has been subjected to softening or semi-softening, to finish working for a length of 100 km, was performed 5 times, and a sample which could be drawn into wire without undergoing wire breakage even for once was rated as "○ (good)", a sample which underwent wire breakage once was rated as "Δ (slightly poor)", and a sample which underwent wire breakage two or more times was rated as "× (poor)".

The hardness of the wire surface section and the wire center section was measured, using a nanoindenter (ENT-2100, manufactured by Elionix, Inc.).

The thickness (µm) of the worked layer on the surface side of the wire was determined from microstructure observation of a wire transverse cross-section (TD cross-section) and the change in hardness in the nanoindenter test, and the thickness was designated as the "surface worked layer thickness (µm)". Furthermore, from this thickness (µm) of the worked layer thus determined, the ratio (%) of the thickness from the outermost surface of the wire to the innermost core side of the worked layer, with respect to the wire diameter φ of wire or the wire thickness t was calculated, and the ratio was designated as the "surface worked layer thickness (%)".

Regarding the coil formability, the frequency of occurrence of wire breakage when 100 km of a copper alloy wire was subjected to coil working into a coil having a diameter of φ 5 mm, was tested, and a sample which did not undergo wire breakage even for once was rated as "○ (good)", a sample which underwent wire breakage once was rated as "Δ (slightly poor)", and a sample which underwent wire breakage two or more times was rated as "× (poor)".

Table 1 shows the results of measuring and evaluating the characteristics of samples of round wires of Examples (Examples 1 to 6) and samples of round wires of Comparative examples (Comparative examples 1 to 7) obtained by working and heating Cu-2% Ag alloy wires to have a final wire diameter of 0.04 mm (φ 40 µm). The conditions for the final-heating (finish-annealing) were changed as indicated in Table 1, and the strength and elongation before the finish cold-working were changed to various values.

As shown in Examples 1 to 6, it is understood that when a copper alloy wire that had been subjected to a final-heating (finish-annealing) so as to have a tensile strength of 330 MPa or more and an elongation of 10% or more, was subjected to finish cold-working at a working ratio of 3 to 15%, a worked layer having a nanoindentation hardness of 1.45 GPa or more was formed in the wire surface section, and the resistance to bending fatigue could be enhanced. Furthermore, as shown in Examples 3 to 5, when the working ratio of the finish cold-working was 7 to 12%, the effect of enhancing the resistance to bending fatigue is superior, and thus it is preferable.

On the contrary, in a case in which the finish cold-working for providing this wire surface section was not carried out as in Comparative example 1, or in a case in which the working ratio for the finish cold-working was too small such as less than 3% as in Comparative example 2 or 3, no worked layer did exist at all, or the layer thickness of the worked layer was so thin that the resistance to bending fatigue could not be enhanced. Furthermore, in a case in which the working ratio of the finish cold-working was too large such as more than 15% as in Comparative example 4 or 5, working proceeded not only on the wire surface section, but also to the entire copper alloy wire including the center side. Thus, the surface worked layer that enhances the resistance to bending fatigue was not satisfactorily formed, the copper alloy wires after the finish cold-working were poor in elongation, and the resistance to bending fatigue could not be enhanced.

Furthermore, in a case in which the final-heating before the finish cold-working is insufficient, and the elongation is less than 10% as in Comparative example 6, the elongation of the copper alloy wire after finish cold-working is less than 7%, and insufficient coil formability is obtained. Furthermore, if softening is carried out excessively as the final-heating before the finish cold-working as illustrated in Comparative example 7, and the tensile strength of the copper alloy wire is less than 330 MPa, the hardness of the wire surface section is insufficient, and the strength after the finish-annealing is also insufficient. Furthermore, wire breakage at the time of finish cold-working is brought about.

Meanwhile, also in the case of rectangular wires, the same results as in the case of the round wires can be obtained.

In Examples 7 to 12 and Comparative examples 8 and 9, the results for evaluating the wire-drawing property when Cu-1% Ag alloy round wires having various diameters obtained by changing the conditions for the final-heating (finish-annealing) as indicated in Table 2, and varying the strength before the finish cold-working to various values, were subjected to finish cold-working at a working ratio of 10%. In Comparative examples 10 and 11, the test was carried out in the same manner as described above, except that Cu-0.3% Ag alloy round wires were used instead of the Cu-1% Ag alloy wires.

For the wire-drawing property, a test of subjecting a copper alloy wire that has been subjected to softening or semi-softening, to finish working for a length of 100 km, was performed 5 times, and a sample which could be drawn into wire without undergoing wire breakage even for once was rated as "○ (good)", a sample which underwent wire breakage once was rated as "Δ (slightly poor)", and a sample which underwent wire breakage two or more times was rated as "× (poor)".

It is understood that in the case of performing wire-drawing on a relatively thick wire with wire diameter φ 0.5 mm or more, wire-drawing can be achieved without any wire breakage; however, in the case of subjecting a wire with diameter φ 0.1 mm or less to wire-drawing, the tensile strength of the copper alloy wire after the finish-annealing before the wire-drawing working is preferably 330 MPa or more. Thus, it is understood that the resistance to bending fatigue can be enhanced, by performing surface working on a fine wire having a diameter of φ 0.1 mm or less, under the production conditions defined in the production method of the present invention.

Meanwhile, also in the case of rectangular wires, the same results as in the case of the round wires can be obtained.

**Table 2**

| | Finish annealing | | | TS after finish heating | Wire-drawability (whether or not breakage in wire-drawing) | | | | | | |
|---|---|---|---|---|---|---|---|---|---|---|---|
| | Manner | Temp. | Time | | Wire diameter (mm) | | | | | | |
| | | °C | | MPa | 0.02 | 0.04 | 0.06 | 0.08 | 0.1 | 0.5 | 1 |
| Ex 7 | Batch | 420 | 30 min | 333 | Δ | Δ | ○ | ○ | ○ | ○ | ○ |
| Ex 8 | Batch | 410 | 30 min | 342 | Δ | ○ | ○ | ○ | ○ | ○ | ○ |
| Ex 9 | Batch | 400 | 30 min | 353 | ○ | ○ | ○ | ○ | ○ | ○ | ○ |
| Ex 10 | Batch | 390 | 30 min | 367 | ○ | ○ | ○ | ○ | ○ | ○ | ○ |
| Ex 11 | Batch | 380 | 30 min | 382 | ○ | ○ | ○ | ○ | ○ | ○ | ○ |
| Ex 12 | Batch | 370 | 30 min | 398 | ○ | ○ | ○ | ○ | ○ | ○ | ○ |
| C ex 8 | Batch | 440 | 30 min | 305 | × | × | × | × | Δ | ○ | ○ |
| C ex 9 | Batch | 430 | 30 min | 325 | × | × | × | × | Δ | ○ | ○ |
| C ex 10 | Batch | 360 | 30 min | 305 | × | × | × | × | Δ | ○ | ○ |
| C ex 11 | Batch | 350 | 30 min | 325 | × | × | × | × | Δ | ○ | ○ |

| | | | | | | | | | | | |
|---|---|---|---|---|---|---|---|---|---|---|---|
| Note: Ex 7 to 12 and C ex 8 to 9: Cu-1%Ag C ex 10 to 11: Cu-0.3%Ag The range enclosed with double-line indicates the working examples according to this invention. | | | | | | | | | | | |

Table 3 shows Examples according to the present invention and Comparative examples of round wires produced from copper alloys of various other alloy compositions. It is understood that when copper alloy wires having a tensile strength of 330 MPa or more and an elongation of 10% or more are produced by a final-heating (finish-annealing) before the finish cold-working, finish cold-working can be performed to obtain a diameter of φ 0.1 mm or less, at a working ratio of 3 to 15%, preferably 5 to 15%, and more preferably 7 to 12%.

Furthermore, it was found that when wires are subjected to predetermined surface working by this finish cold-working at a working ratio of 3 to 15%, preferably 5 to 15%, and more preferably 7 to 12%, the resistance to bending fatigue of the copper alloy wires can be enhanced, and a magnet wire having sufficient coil formability with an elongation after finish cold-working of 7% or more, and preferably 10% or more, and having a long coil service life can be obtained.

Particularly, from a comparison between Comparative examples and Examples according to the present invention, it is understood that when the nanoindentation hardness in a depth region extending from the outermost surface of the wire toward at least 5% inner side in the wire diameter is 1.45 GPa or more, and the final wire has a tensile strength of 350 MPa or more and an elongation of 7% or more, desired physical properties can be achieved.

Table 4 shows Examples according to the present invention and Comparative examples of rectangular wires produced from copper alloys of various alloy compositions. From the results shown in Table 4, also in the case of rectangular wires, the same results as in the case of the round wires can be obtained.

## Claims

1. A copper alloy wire, having an alloy composition consisting of (i) 0.5 to 4 mass% of Ag and/or (ii) at least one selected from the group consisting of Sn, Mg, Zn, In, Ni, Co, Zr, and Cr each at a content of 0.05 to 0.3 mass%, with the balance being Cu and unavoidable impurities,
wherein the copper alloy wire has a wire diameter or a wire thickness of 0.1 mm or less, and
wherein the nanoindentation hardness in the wire surface section is 1.45 GPa or more as measured by nanoindenter ENT-2100 (manufactured by Elionix, Inc.), the wire surface section starting at the outermost surface of the wire and ranging at maximum to a distance from the surface that corresponds to 20% of the wire diameter or the wire thickness; the nanoindentation hardness at the center of the wire is less than 1.45 GPa as measured by nanoindenter ENT-2100 (manufactured by Elionix, Inc.), the tensile strength of the wire is 350 MPa or more, and the elongation of the wire is 7% or more.

2. A method for producing the copper alloy wire of claim 1, containing the steps of:
wire-working of subjecting a rough-drawn wire of a copper alloy having an alloy composition consisting of (i) 0.5 to 4 mass% of Ag and/or (ii) at least one selected from the group consisting of Sn, Mg, Zn, In, Ni, Co, Zr, and Cr each at a content of 0.05 to 0.3 mass%, with the balance being Cu and unavoidable impurities, to cold-working, to form a wire having a wire diameter or a wire thickness of 0.1 mm or less;
final-heating, which is carried out in a batch mode at 300°C to 450°C for 30 minutes to 2 hours, or in a continuous mode at 300°C to 700°C for 0.5 to 5 seconds; and
cold-working the wire that has been subjected to the heating, at a working ratio of 3 to 15%.

3. The method for producing a copper alloy wire according to claim 2, wherein in the wire-working step, intermediate heating is carried out in the course of a plurality of cold-working steps so that the wire after this intermediate heating has a tensile strength of 330 MPa or more and an elongation of 10% or more.

## Patentansprüche

1. Draht aus Kupferlegierung, der eine Legierungszusammensetzung aufweist, die aus (i) 0,5 bis 4 Masse-% Ag und / oder (ii) mindestens einem, das aus der Gruppe, welche aus Sn, Mg, Zn, In, Ni, Co, Zr und Cr besteht, jedes davon in einem Gehalt von 0,05 bis 0,3 Masse-%, ausgewählt ist, besteht, wobei der Rest Cu und unvermeidbare Verunreinigungen sind,
wobei der Draht aus Kupferlegierung einen Drahtdurchmesser oder eine Drahtdicke von 0,1 mm oder weniger aufweist, und
wobei die Nanoindentationshärte in einem Oberflächenabschnitt des Drahts 1,45 GPa oder mehr beträgt, gemessen mit Hilfe von einem Nanoindenter ENT-2100 (hergestellt von Elionix, Inc.), wobei der Oberflächenabschnitt des Drahts an der äußersten Oberfläche des Drahts beginnt und maximal bis zu einem Abstand von der Oberfläche reicht, der 20% des Drahtdurchmessers oder der Drahtdicke entspricht; die Nanoindentationshärte in der Mitte des Drahtes weniger als 1,45 GPa, beträgt, gemessen mit Hilfe von einem Nanoindenter ENT-2100 (hergestellt von Elionix, Inc.); die Zugfestigkeit des Drahtes 350 MPa oder mehr beträgt, und wobei die Dehnung des Drahts 7 % oder mehr beträgt.

2. Verfahren zur Herstellung des Drahts aus Kupferlegierung nach Anspruch 1, welches die folgenden Schritte enthält:
Drahtbearbeitung, wobei ein vorgezogener Draht aus einer Kupferlegierung, der eine Legierungszusammensetzung aufweist, die aus (i) 0,5 bis 4 Masse-% Ag und / oder (ii) mindestens einem, das aus der Gruppe, welche aus Sn, Mg, Zn, In, Ni, Co, Zr und Cr besteht, jedes davon in einem Gehalt von 0,05 bis 0,3 Masse-%, ausgewählt ist, besteht, wobei der Rest Cu und unvermeidbare Verunreinigungen sind, einer Kaltbearbeitung unterzogen wird, um einen Draht zu bilden, der einen Drahtdurchmesser oder eine Drahtdicke von 0,1 mm oder weniger aufweist;
abschließendes Erwärmen, das im Chargenmodus bei 300 °C bis 450 °C für 30 Minuten bis 2 Stunden durchgeführt wird; oder in einem kontinuierlichen Modus bei 300 °C bis 700 °C für 0,5 bis 5 Sekunden durchgeführt wird; und
Kaltbearbeitung des Drahts, der der Erwärmung unterzogen worden ist, bei einem Verarbeitungsverhältnis von 3 bis 15 %.

3. Verfahren zur Herstellung eines Drahts aus einer Kupferlegierung nach Anspruch 2, wobei im Schritt der Drahtbearbeitung eine Zwischenerwärmung im Verlauf einer Vielzahl von Schritten der Kaltbearbeitung durchgeführt wird, so dass der Draht nach dieser Zwischenerwärmung eine Zugfestigkeit von 330 MPa oder mehr und eine Dehnung von 10% oder mehr aufweist.

## Revendications

1. Fil en alliage de cuivre ayant une composition d'alliage se composant de (i) 0,5 à 4 % en poids de Ag et/ou (ii) d'au moins un élément sélectionné dans le groupe consistant en Sn, Mg, Zn, In, Ni, Co, Zr et Cr chacun à une teneur de 0,05 à 0,3 % en poids, avec le reste constitué par Cu et les impuretés inévitables,
dans lequel le fil en alliage de cuivre a un diamètre de fil ou une épaisseur de fil de 0,1 mm ou moins, et
dans lequel la dureté de nanoindentation dans la section de surface de fil est de 1,45 GPa ou plus, telle que mesurée par le nanopénétrateur ENT-2100 (fabriqué par Elionix, Inc.), la section de surface de fil commençant au niveau de la surface située le plus à l'extérieur du fil et s'étendant au maximum à une distance de la surface qui correspond à 20 % du diamètre de fil ou de l'épaisseur de fil ; la dureté de nanoindentation, au centre du fil, est inférieure à 1,45 GPa, telle que mesurée par le nanopénétrateur ENT-2100 (fabriqué par Elionix, Inc.), la résistance à la traction du fil est de 350 MPa ou plus, et l'allongement du fil est de 7 % ou plus.

2. Procédé pour produire le fil en alliage de cuivre selon la revendication 1, comprenant les étapes suivantes :
travailler le fil en soumettant un fil grossièrement tréfilé d'un alliage de cuivre ayant une composition d'alliage se composant de (i) de 0,5 à 4 % en poids de Ag et/ou (ii) au moins un élément sélectionné dans le groupe se composant de Sn, Mg, Zn, In, Ni, Co, Zr et Cr chacun à une teneur de 0,05 à 0,3 % en poids, avec le reste constitué par Cu et les impuretés inévitables, au travail à froid, pour former un fil ayant un diamètre de fil ou une épaisseur de fil de 0,1 mm ou moins ;
le chauffage final, qui est réalisé dans un mode différé de 300 °C à 450 °C pendant 30 minutes à 2 heures, ou dans un mode continu de 300 °C à 700 °C pendant 0,5 à 5 secondes ; et
travailler à froid le fil qui a été soumis au chauffage, à un rapport d'usinage de 3 à 15 %.

3. Procédé pour produire un fil en alliage de cuivre selon la revendication 2, dans lequel à l'étape du travail du fil, le chauffage intermédiaire est réalisé au cours d'une pluralité d'étapes de travail à froid de sorte que le fil, après ce chauffage intermédiaire, a une résistance à la traction de 330 MPa ou plus et un allongement de 10 % ou plus.
